

## UNITED STATES PATENT OFFICE

2,120,377

## MANUFACTURE OF ASPHALTS

Vladimir L. Shipp, New York, Arthur H. Boenau, Sunnyside, and James W. Ramsay, New York, N. Y., assignors to Socony-Vacuum Oil Company, Incorporated, New York, N. Y., a corporation of New York

No. Drawing. Application March 6, 1937,  
Serial No. 129,376

## 14 Claims. (CL. 196—13)

This invention relates to asphaltic products of the kind suitable for paving and similar purposes and relates especially to methods of producing such products. The invention relates particularly to the production of such asphaltic products from petroleum.

It is customary to define the characteristics and properties of asphaltic materials by means of measurements and ratios, such as penetration and ductility values, melting points, and temperature susceptibilities, the latter being represented by the ratio of penetrations at various temperatures, for instance, at 100° F. and 77° F. or at 77° F. and 32° F. These measurements are made by standard methods of test of the American Society for Testing Materials. For example, penetration values are obtained by measuring the distance of penetration of various asphaltic materials by a specified needle loaded with a specified weight at a specified temperature for a specified time (see A. S. T. M. method No. D5—25, Penetration of Bituminous Materials). Ductility values are obtained by measuring the elongation before breaking of a specified sample pulled apart at a specified speed and at a specified temperature (see A. S. T. M. tentative method No. 4, D113—32T, Ductility of Bituminous Materials). Melting points (softening points) are commonly determined by the ball and ring method, which consists in filling a ring with asphalt and placing a steel ball of specified weight in the center of the asphalt, and then gradually heating the asphalt by means of hot water. The melting point is recorded as the temperature at which the asphalt, under the load of the ball, touches the bottom of the water bath (see A. S. T. M. method No. D36—26, Softening Point for Bituminous materials). The above methods are used for the determinations given herein.

The properties represented by the above measurements are important from the standpoint of the present invention. It is important that asphaltic products employed for the purposes contemplated herein be of proper hardness, as determined by penetration tests, and that they be of low temperature susceptibility and of high ductility. Penetration is a measure of consistency and hardness, serving primarily to classify asphalt into commercial grades of various degrees of hardness. Temperature susceptibility (penetration ratio) indicates the susceptibility of a product to change of hardness with change in temperature, that is, its rate of softening. It is desirable that temperature susceptibility as ex-

pressed by the above indicated ratio be as low as possible, since, if it is too high, those asphalts which have suitable hardness for cold weather will flow and be deformed in warm weather and, conversely, those suitable for warm weather will be too brittle for cold weather use. Ductility is a measure of the cementing power of asphaltic material, that is, its power to hold together the aggregate or other mineral filler in the final pavement compound, and is a very desirable property, contributing extensively to the ability of pavements and similar asphaltic structures to withstand wear, disintegration, traffic shock, mechanical stresses due to temperature, weathering, and the like. For example, asphalts having low ductility, when used in paving mixtures, produce mixtures which separate and disintegrate under conditions of use, while asphalts of high ductility are capable of absorbing more filler than ordinary asphalts without objectionably impairing the mechanical strength of the mixture.

The importance of the above properties in asphaltic material may be illustrated by the specifications and requirements of the State of Texas and the city of New York which are here reproduced in part:

## STATE OF TEXAS

| Grade    | Penetration<br>@ 77° F.<br>100 grams<br>5 seconds | Penetration<br>@ 32° F.<br>200 grams<br>60 seconds | Ductility<br>@ 77° F. cms. | Melting<br>point<br>(° F.) of | 30 |
|----------|---------------------------------------------------|----------------------------------------------------|----------------------------|-------------------------------|----|
| OA 230-T | 210-250                                           | 50 minimum                                         | 50 minimum                 | 86-122                        | 35 |
| OA 90    | 85-100                                            | 30 minimum                                         | 50 minimum                 | 113-140                       |    |
| OA 55    | 50-60                                             | 22 minimum                                         | 50 minimum                 | 113-140                       |    |
| OA 45    | 40-50                                             | 18 minimum                                         | 40 minimum                 | 113-140                       |    |

## CITY OF NEW YORK

## ASPHALTIC CEMENT (TENTATIVE 24-A-7A) 40

## Penetration

At 32° F., 100 grams, 5 sec.—Not less than 3.  
At 77° F., 100 grams, 5 sec.—30-40, 40-50, 50-60 or 60-70 as called for.

At 100° F., 100 grams, 5 sec.—Not more than 4 times that at 77° F. 45

## Ductility

At 77° F., not less than 40 centimeters at 50 penetration. 50

## JOINT FILLER

## Penetration

At 32° F., 100 grams, 5 sec.—Minimum 4.

At 77° F., 100 grams, 5 sec. 60-100. 55

At 100° F., 100 grams, 3 sec.—Maximum 3.25 times that at 77° F.

#### Ductility

5 At 77° F., not less than 40 centimeters.

Up to the present time, commercial manufacture of petroleum asphalt has been largely dependent upon the fortuitous presence of desirable properties in selected crude oils for the attainment of characteristics such as described and specified above; i. e., asphaltic or naphthenic crudes or asphaltic or naphthenic residues from mixed base crudes. Such crudes, roughly in the order of their desirability, are Mexican, Venezuelan, Smackover, Californian, and Coastal. The best stocks; e. g., Mexican, can be steam refined to produce asphalts, but for those grades of asphalt requiring low temperature susceptibility, as typified by the above specifications, the stocks must be air blown. Blowing results in loss of ductility. This tendency sometimes may be minimized to a limited extent by careful operation, but with a great many residual oils capable of being converted into otherwise desirable asphalts by blowing, no amount of care will serve to produce products of desirable ductility. In order to obtain satisfactory ductility in asphalts requiring low temperature susceptibility, resort must be made to a very careful selection of crudes, even among the best Mexican and Venezuelan stocks, it being almost impossible to produce desired grades from domestic crudes.

It is an important object of the present invention to produce from commonly available petroleum stocks asphalt products which combine the above described desired properties, such as high ductility and low temperature susceptibility, and which are especially suitable for use in road surfaces and the like. It is an object to produce petroleum asphaltic products to meet specifications as desired without dependence upon the use of particular natural asphaltic stocks of specially selected quality. These objects are accomplished, and a novel product is produced, by a simple low cost novel process.

The present invention is based upon the discovery that asphaltic products having desirable properties, as above described, can be produced by blowing certain solvent tars to effect conversion of the more naphthenic portions of the oil content of the tar into asphaltic material, and then adding to the blown tar an oil whose V. I. (viscosity index—see article by Dean and Davis, Chemical and Metallurgical Engineering, October 1929, pages 618 and 619) is substantially higher than that of the oil which has been removed from the oil content of the tar by the aforesaid conversion.

60 It has been proposed to make asphaltic products by blowing solvent tars, but asphalts so produced are dependent for their properties upon the character of the tar employed,—the same as asphalts have been dependent upon the character of the crude oil used,—and solvent tar asphalts as a class are characterized by notably poor temperature susceptibility and are therefore inferior and unsuitable for the uses contemplated herein. 65 It has also been proposed to precipitate relatively oil-free bitumens from petroleum residues or petroleum asphaltic products with a precipitant such as propane, and then add back to the precipitated bitumens oils of desired properties to produce asphalt products. This process is compli-

cated, slow and costly. The separated bitumens also are not in fact oil-free, and any oil that they contain is the more naphthenic portion of the oil content of the original material to which the propane precipitant was added, the more paraffinic portions having gone off with the propane. 5

The present invention, on the other hand, produces asphalts of good properties, controlled as desired, including high ductility, good (low) temperature susceptibility, and good penetration, 10 and accomplishes this without necessity of removing any portion of the material by costly steps of solvent precipitation, vacuum distillation, or the like. In the present invention a portion of the oil content of the solvent tar is removed by conversion into asphaltic material, which is less expensive than removal by solvents or precipitants, increases yield of asphalt, reduces oil content, and effects such reduction in oil content by getting rid of the highly naphthenic portion of the oil content which would be the most objectionable in the asphalt and is not wanted. That is, in the present invention, and contrary to what occurs when propane precipitation is employed, the more naphthenic portions of the oil 25 content of the tar are removed first by conversion into asphaltic material, the unconverted portions being less naphthenic and therefore more desirable in the asphalt. This increases yield and improves temperature susceptibility by improving 30 the V. I. of the remaining oil content of the asphalt. Temperature susceptibility is then further improved by adding additional oil of appropriately high V. I. This invention also makes it possible to take advantage of the high ductility 35 characteristic of solvent tar asphalts, and at the same time and at low cost to combine this property with good temperature susceptibility in a finished asphalt.

The preferred classes of solvent tars suitable 40 for the uses of this invention are naphthenic tars resulting from the single or double solvent extraction of long or short residuums from asphaltic or mixed base crudes, employing naphthenic solvents of the class typified by cresylic 45 acid, phenol, furfural, nitrobenzene, sulfur dioxide, and the like, or the substantial equivalent of such tars. However, although it is preferable to utilize solvent tars of relatively high asphaltic content and less asphaltic tars are relatively less 50 useful, less asphaltic tars can be used to some extent and also can be reduced by distillation to obtain useful residues of fairly high asphaltic content, and can then be exposed to the steps of the process described herein. It is the class of 55 solvent tars defined herein that is covered by the term as used in the claims. These tars are not the same or equivalent to propane precipitated bitumens. These solvent tars normally and preferably contain some asphaltic matter before 60 blowing; i. e., asphaltenes and resins. They also contain oil. The greater proportion of the oil content of the tars is highly naphthenic and readily forms asphaltic matter upon blowing. The most naphthenic portions; i. e., the oil that would be the most undesirable in the finished asphalt, is the most unstable and therefore is the first to be removed by conversion upon blowing. The oils contained in solvent tars have very low 65 viscosity indices, as they include a large proportion of highly naphthenic constituents. The viscosity indices of these oils are far below zero on the standard 0-100 viscosity index scale. It is the presence of these highly naphthenic or low 70

75

viscosity index oils which to a great extent imparts a high temperature susceptibility to asphalts derived from solvent tars. In the present invention the oils present in solvent tars are selectively converted and/or removed by blowing the tars with air or other oxidizing gas to a controlled extent, followed by addition of oil of better V. I. By proceeding in this manner the most undesirable naphthenic constituents are removed while the more paraffinic oils remain, thereby producing an oil content of improved viscosity index.

The oil content of the solvent tars is usually so highly naphthenic that the blowing operation is in itself not capable of producing an asphalt of sufficiently low temperature susceptibility. It is therefore an important step in the present invention to add suitable amounts of relatively paraffinic oils to the blown tar; i. e., oils of relatively high viscosity index as compared with the original oil content of the solvent tar. The quantity and degree of paraffinicity of these added oils can be varied with the result that the process can be easily controlled both as to extent of blowing and the amount and character of oil addition. Ordinarily the added oil will have not only a higher viscosity index than that of the oil originally present in the tar, but will have a viscosity index higher than that of the improved oil remaining in the tar after the blowing treatment. Because of the extremely low V. I. of the oil content of the solvent tars, good temperature susceptibility improvement can ordinarily be obtained with diluent oils ranging down to zero V. I. The viscosity of the oil added to the solvent tar does not materially affect the quality of the final asphalt, but light oil, just passing flash point requirements and the like, is ordinarily used, because such oil is cheaper than more viscous oil and less of it is required to bring the asphalt to proper penetration.

The solvent tar may be blown to any suitable extent, as desired, but is preferably blown to a point beyond the penetration and/or melting point specifications desired in the finished asphalt, and is then brought back to the desired or specified values by adding oil of proper viscosity index characteristics, which causes a definite improvement or lowering of the temperature susceptibility for the specified penetration value or melting point. The blowing is conducted at elevated temperatures, say 400°-500° F., in the known manner of asphalt blowing. As a specific example of this manner of proceeding, the solvent tar may be blown to a penetration value of 30 at 77° F., and may then be cut back with a suitably high viscosity index oil to lower the temperature susceptibility and raise the penetration value to commercially useful grades, the hardest commercial grade having a penetration value of about 40 at 77° F. The solvent tar may be blown to the point of apparent loss of ductility, i. e., to a point where the ductility is so low that it records as zero on the ductility testing machine, and then the ductility and penetration values can be raised by the addition of the oil of suitably high viscosity index. In such a case, the upper limit of hard blowing is where the ductility is too low even after adding the oil to the blown tar, which ordinarily occurs when the tar is blown to a melting point of about 220° F.

As examples illustrative of the invention, the following data are given showing four different asphalt products embodying the invention.

### Composition

|                                                              | Percent | Percent | Percent | Percent |
|--------------------------------------------------------------|---------|---------|---------|---------|
| Solvent tar blown—<br>to 156° F., M. P.<br>to 170° F., M. P. |         |         |         | 87.5    |
| Blending oil No. 1                                           | 86.0    | 81.5    | 88.2    | 12.5    |
| Blending oil No. 2                                           | 14.0    | 18.5    | 13.8    |         |

5

10

### Properties

|                                   | Percent | Percent | Percent | Percent |
|-----------------------------------|---------|---------|---------|---------|
| Melting point (R. & B.),<br>° F.  |         |         |         | 115.5   |
| Pen. @ 77° F., 100 g.,<br>5 sec.  | 125     | 115     | 124.5   |         |
| Pen. @ 32° F., 100 g.,<br>5 sec.  | 53      | 103     | 60      | 95      |
| Pen. @ 32° F., 200 g.,<br>60 sec. | 4       | 8       | 6       | 7       |
| Ductility @ 77° F., cms.          | 20      | 32      | 23      | 36      |
|                                   | 100+    | 100+    | 100+    | 100+    |

15

20

25

30

In the above examples blending oil No. 1 is a distillate derived from mixed base crude having an A. P. I. gravity of 25.9°, flash C. O. C. 365° F., S. U. viscosity 113.6 at 100° F., and viscosity index 75. Blending oil No. 2 is a gas oil distillate from an asphaltic base crude of A. P. I. gravity 21.3°, flash C. O. C. 335° F., S. U. viscosity 144 at 100° F., and viscosity index 25.

We claim:

1. A process for manufacturing an asphaltic material which comprises air blowing a solvent tar to convert a portion of its naphthenic oil content into asphaltic material, and adding to said blown tar an oil of viscosity index higher than the viscosity index of the original naphthenic oil content of the solvent tar.

2. A process for manufacturing an asphaltic material of high ductility and low temperature susceptibility which comprises air blowing a solvent tar at elevated temperature to convert the more naphthenic portions of the oil content of said tar into a more asphaltic material, leaving the less naphthenic portions unconverted, and improving the temperature susceptibility by adding to said blown tar an oil less naphthenic than the remaining naphthenic oil content of the blown solvent tar.

3. The method of making asphalt which comprises altering the more naphthenic portion of the oil content of a solvent tar by oxidizing same into asphaltic material, and replacing said removed portion with an oil less naphthenic than the oil which was oxidized.

4. A process for obtaining an asphaltic material having a low susceptibility ratio and a high ductility value which comprises obtaining a solvent tar containing an oil of a low viscosity index by solvent refining a petroleum product containing naphthenic constituents, oxidizing the more naphthenic portion of said tar into asphaltic matter while leaving the less naphthenic portion unconverted, and adding to said tar an oil having a viscosity index higher than the viscosity index of said first named oil.

5. A process for obtaining an asphaltic material having a low susceptibility ratio and a high ductility value which comprises solvent refining a petroleum residue to obtain a solvent tar containing oils of low viscosity index, air blowing said tar until a major portion of said oils is oxidized while leaving a minor portion of oil which has a higher viscosity index than the oil which was oxidized, and adding to the blown tar an oil of

50

45

55

60

65

70

75

- higher viscosity index than that of said remaining unconverted portion of oil.
6. A process for manufacturing an improved asphaltic material which comprises solvent refining a petroleum residue to obtain a solvent tar, air blowing said tar to an excessively low penetration value and an excessively high melting point, and adding an oil of relatively high viscosity index to said air blown tar, thereby 5 raising the penetration value and lowering the melting point of the tar-oil mixture to predetermined desirable values and simultaneously lowering the susceptibility ratio of said mixture below that normally existing in said tar at said 10 values.
7. A process for manufacturing an improved asphaltic material which comprises solvent refining a petroleum residue to obtain a solvent tar, air blowing said tar to a penetration value of not 20 more than 30 at 77° F., and adding an oil of relatively high viscosity index to said air blown tar, thereby raising said penetration value to a predetermined desirable value not less than 40 at 77° F. and simultaneously lowering the susceptibility 25 ratio of the tar-oil mixture below that normally existing in said tar at said predetermined value.
8. A process for manufacturing an improved asphaltic material which comprises solvent refining a petroleum residue to obtain a solvent tar, air blowing said tar to a point of apparent loss of ductility and to an excessively low penetration value, and adding an oil of relatively high viscosity index to said air blown tar, thereby 30 raising said ductility and penetration values to predetermined desirable values and simultaneously lowering the susceptibility ratio of the tar-oil mixture below that normally existing in said tar at said predetermined values.
- 40 9. A process for manufacturing an improved asphaltic material which comprises distilling solvent tars having a relatively low asphaltic content to produce a tar having a relatively high asphaltic content, said tar containing an oil of 45 relatively low viscosity index, air blowing said
- tar, and adding an oil of relatively high viscosity index to said blown tar.
10. The method of making asphalt of high ductility and low penetration ratio which comprises air blowing a solvent tar to an asphalt of 5 substantially zero ductility, and adding to said hard blown tar an oil of viscosity index higher than that of the oil content of the solvent tar before blowing.
11. An improved asphaltic material comprising 10 an air blown solvent tar asphalt and an oil of viscosity index higher than that of the oil content of the solvent tar prior to air blowing.
12. An improved asphaltic material comprising 15 an air blown solvent tar and an oil of relatively high viscosity index, said air blown tar being free of oil of the nature of the more naphthenic portion of the oil present in the tar prior to air blowing.
13. An improved asphaltic material having a 20 relatively high ductility value and a relatively low susceptibility ratio comprising an air blown solvent tar and an oil of relatively high viscosity index not less than 0, said air blown tar containing a small portion of an oil of relatively low viscosity index which was present in the tar prior 25 to blowing.
14. A petroleum asphalt product comprising naturally occurring asphaltic matter extracted from petroleum, synthetic asphaltic oxidation 30 products of the more naphthenic portion of the oil content of a naphthenic solvent extract, oil which is the less naphthenic portion of the oil content of the aforesaid naphthenic solvent extract, and an additional oil of higher viscosity 35 index than the oil content of said naphthenic solvent extract, the second named constituent having been produced by oxidizing a solvent tar which also contained the first and third named constituents, and the last named constituent 40 having been added to the oxidized tar.

VLADIMIR L. SHIPP.  
ARTHUR H. BOENAU.  
JAMES W. RAMSAY. 45